# EUROPEAN PATENT SPECIFICATION

(11) **EP 1 461 483 B1**
(45) Date of publication and mention of the grant of the patent: **04.04.2007**
(21) Application number: 02801025.4
(22) Date of filing: 11.10.2002
(51) Int. Cl.: D04H 1/46, D04H 3/10

(54) **DIFFERENTIALLY ENTANGLED NONWOVEN FABRIC FOR USE AS WIPES**
DIFFERENTIELL VERWIRBELTER VLIESSTOFF ALS WISCHTUCH
TISSU NON TISSE A ENCHEVETREMENTS DE FIBRES DIFFERENTS DESTINE A ETRE UTILISE COMME LINGETTE

(30) Priority: 12.10.2001 US 329214 P
(43) Date of publication of application: 29.09.2004
(73) Proprietor: Polymer Group, Inc., North Charleston, SC 29406 (US)
(72) Inventor: FULLER, Charles, Kannapolis, NC 28081 (US); LEDBETTER, Sheridan, Maumelle, AR 72113 (US); MERCER, Steve, Benton, AR 72015 (US); CAMPBELL, Willie, J., Jr., Benson, NC 27504 (US)
(74) Representative: Lyons, Andrew John
(86) International application number: PCT/US2002/032498
(87) International publication number: WO 2003/031710

(56) References cited:
- EP-A- 0 473 325
- EP-A- 0 602 881
- WO-A-01/59194
- WO-A-02/31249
- WO-A-98/23804
- US-A- 3 485 706
- US-A- 4 647 490
- US-A- 5 106 457
- US-A- 5 801 107

## Description

### Technical Field

The invention disclosed herein is directed to wipes, preferably wipes for use in graphic arts or lithography, made from a hydroentangled nonwoven fabric, whereby the outer surface fibers of a single fibrous batt are highly hydroentangled and the inner fibers of the single fibrous batt are lightly entangled, the resulting fabric thus exhibits a low linting, lofty structure, and favorable tactile and ductile softness while obtaining sufficient physical strength.

### Background of the Invention

The use of natural fiber materials in industrial applications has been found to be highly advantageous in situations where a non-linting, absorbent pad or wiper is required. A material that has been employed in such applications is found in the Webril material from the Kendall Company of Massachusetts. The Webril material is a compressed, mercerized cotton fibrous batt. The mercerization process involves the swelling of the natural cotton's ribbon like profile into an approximately round profile of larger diameter. Typically, caustic washes are utilized while the cotton batt is under tension to induce the swelling of the cotton fiber. Because of the use of a caustic solution, it is necessary to subsequently treat the cotton material with an acidic solution so as to neutralize the material and render it useable. A number of complicated steps are required to successfully perform the process, with a significant amount of environmentally harmful effluent being produced.

In the interest of forming natural fiber nonwoven pads or wipers without the by- products of mercerization, the application of a resin binder in conjunction with hydroentanglement was explored as evidenced by U.S. Patents No. 2,862,251, No. 3,033,721, No. 3,769,659, and No. 3,931,436 to Kalwaites et al., and U.S. Patents No. 3,081,515 and No. 3,025,585 to Griswold et al. The application of resin binder was found to have a deleterious effect on the softness of the corresponding nonwoven fabric.

The findings by Evans, U.S. Patent No. 3,485,706 suggested that the impedance of energetic water streams on a fibrous batt could produce a nonwoven fabric by the entanglement of those fibers with one another through the depth of the fibrous batt, thus obviating the need for a resin binder. However, the action of the water streams upon the fibrous batt and the action of entangling the fibers result in a fabric having significantly decreased bulk, and correspondingly decreased tactile and ductile softness.

Various attempts have been made in order to obtain a durable natural fiber nonwoven fabric while maintaining sufficient strength and softness. In U.S. Patent No. 5,849,647 to Neveu, a hydrophilic cotton stratified structure is formed by interceding an air-randomized core in between two previously formed, highly fiber oriented carded layers. The stratified layers are subsequently treated with a soda liquor which is then boiled off to render an integrated structure. While a cotton structure performed by the manner described can render an ultimate material that is low linting, the material must undergo substantial processing in the forming of separate and distinct layers and the juxtaposition of those layers during the caustic integration step. U.S. Patent No. 4,647,490 to Bailey et al., formed an apertured, cotton fiber nonwoven material by hydroentanglement induced by oscillating water streams. In the Bailey process, the fibers of the fibrous batt are washed down and through the fibrous batt in order to entangle the fibers and form apertures in the fabric. U.S. Patent No. 4,426,417 to Meitner et al., incorporated the use of thermoplastic meltblown during the formation of a fibrous batt as a means for attaining the loft for absorbency and maintain sufficient physical strength by bonding the fibers together. As the nature of the Meitner process is based upon the total and effective binding of the fibers to the thermoplastic meltblown there are potential issues with unbound or loosely bound fibers being disengaged from the meltblown.

WO02/31249A discloses a nonwoven fabric comprising a single fibrous batt whereupon the single fibrous batt is entangled by the application of hydraulic energy in the range of 0.027 to 0.046 hp-hr/lb to form a nonwoven fabric, said nonwoven fabric having a highly entangled outer surface region and a lightly entangled inner core region.

EP-A-0602881 discloses a nonwoven wipe comprising a single fibrous batt whereupon the single fibrous batt is entangled by the application of hydraulic energy. WO98/23804A and EP-A-0473325 disclose similar wipes.

Given the prior art attempt to form a nonlinting, soft and yet strong absorbent materials, there remains a need for a nonwoven fabric exhibiting these characteristics and yet is formed in an expeditious and uncomplicated manner.

A method for forming a suitable nonwoven fabric meeting the aforementioned requirements has been identified in the application of fluidic energy such that a single fibrous batt is imparted with a highly entangled surface of outer fibers while retaining the loft and absorbency of a lightly entangled central layer of core fibers.

### Summary of The Invention

The present invention is directed to a method of forming a nonwoven fabric, the outer surface of which exhibits highly entangled fibers whereas the inner layer exhibits lightly entangled fibers. In particular, the present invention contemplates that a fabric is formed from a fibrous batt that is subjected to fluidic energy, preferably hydraulic energy, applied to one or both faces of a fibrous batt. The hydraulic energy is moderated against the basis weight of the fibrous batt to achieve the degree of surface entanglement desired.

In accordance with the present invention, there is provided a nonwoven wipe, comprising a single fibrous batt whereupon the single fibrous batt is formed from fibers selected from 100% cotton fibers and a blend of cotton and synthetic staple length fibers, and is entangled by the application of hydraulic energy in the range of about 233.4 to 350.1 J/g (0.040 to 0.060 hp.hr/lb.) to form a differentially entangled nonwoven wipe, said nonwoven wipe having a highly entangled outer surface region and a lightly entangled inner core region, wherein said highly entangled region and said lightly entangled region are each formed from the one of said selected fibers, subject to the proviso that the hydraulic energy applied is more than 268.4 J/g (0.046 hp.ht/lb.)

While use of natural fibers is common, the fibrous matrix, may comprise synthetic fibers or blends of natural and synthetic fibers. The synthetic fibers are chosen from the group consisting of viscose cullulose, polyacrylates, polyolefins, polyamides, polyesters and combinations thereof. Further, the synthetic fibers may comprise homogeneous, bicomponent and/or multi-component profiles, and the blends thereof.

In a particularly preferred form, the fibrous batt is carded and cross-lapped to form a fibrous batt. The fibrous batt is then continuously indexed through a station composed of a rotary foraminous surface and a fluidic manifold. Fluid streams from the fluidic manifold impinge upon the fibrous batt at a controlled energy level so as to integrate a portion of the overall fibrous content. The energy level is controlled such that the energy is sufficient to induce high levels of entanglement in the surface fibers, but has insufficient transmitted energy to induce high levels of entanglement of the inner fibers. A plurality of such stations can be employed whereby fluid streams are at the same or differing energy levels, impinging one or alternately both surfaces of the fibrous batt. The resulting differentially entangled nonwoven web exhibits a highly entangled fibrous outer surface and a lightly entangled fibrous core.

Subsequent to hydroentanglement, the present method further contemplates the provision of a three-dimensional image transfer device having a movable imaging surface. Such three-dimensional image transfer devices are disclosed in U.S. Patent No 5,098,764. In a typical configuration, the image transfer device may comprise a drum-like apparatus that is rotatable with respect to one or more hydroentangling manifolds.

It is within the purview of this invention that tension control means can be employed to further enhance the physical performance of the resulting lofty material.

A further aspect of the present invention is directed to a method of forming a nonwoven fabric which exhibits a sufficient degree of softness and nonlinting performance, while providing the necessary resistance to tearing and abrasion, to facilitate use in a wide variety of applications. The fabric exhibits a high degree of loft and absorbency, thus permitting its use in those applications in which the fabric is applied as a cleaning wipe. Further, the material exhibits pleasant aesthetics, thus lending itself to application in medical applications.

A method of making the present durable nonwoven fabric comprises the steps of providing a fibrous matrix or batt, which is subjected to controlled levels of hydraulic energy. A homogeneous cotton fibrous batt has been found to desirably yield a fabric with soft hand and good absorbency. The fibrous batt is formed into a differentially entangled nonwoven fabric by the application of sufficient energy to entangle only the outer layers of the fibrous batt. Subsequently, the fabric can be passed over an image transfer device defined by three-dimensional elements against which the differentially entangled nonwoven fabric is forced during further application of further energy, whereby the fibrous constituents of the web are imaged and patterned by movement into regions between the three-dimensional elements of the transfer device.

It is within the purview of the present invention that physical property altering chemistries can be incorporated into the resulting differentially entangled fabric. Such chemistries include for example antimicrobial and antistatic agents that can be durably applied to the constituent fibers of the fibrous batt, to the fibrous batt during manufacture, and/or to the resulting fabric.

Other features and advantages of the present invention will become readily apparent from the following detailed description, the accompanying drawings, and the appended claims.

### Brief Description Of The Drawings

FIGURE 1 is a diagrammatic view of an apparatus for manufacturing a differentially entangled nonwoven fabric, embodying the principles of the present invention; and
FIGURE 2 is a diagrammatic view of five consecutive entangling sections and an image transfer station.

### Detailed Description

While the present invention is susceptible of embodiment in various forms, there is shown in the drawings and will hereinafter be described a presently preferred embodiment of the invention, with the understanding that the present disclosure is to be considered as an exemplification of the invention, and is not intended to limit the invention to the specific embodiment illustrated.

The present invention is directed to a method of forming nonwoven fabrics by hydroentanglement, wherein the outer surface of the fabric is substantially more entangled than the core layer. Hydroentanglement by this method is controlled by the application of fluidic energy such that the energy imparted into fibers of the fabric is sufficient to highly entangle only the outer fibers. The inner fibers are lightly entangled such that the overall structure is resistant to separation of the layers, yet retain much of the loftiness or bulk of the fibrous core layer that is responsible for tactile and ductile softness as well as absorbency. By advancing the fibrous batt with a relatively low tension through one or more entanglement stations, differential fiber entanglement is achieved, with the physical properties, both aesthetic and mechanical, of the resultant fabric being desirably achieved.

In accordance with a further aspect of the present invention, a nonwoven fabric for application as a wipe can be produced such that the level of surface entanglement can be controlled resulting in surface layers that are extremely resistant to linting while the fabric retains some loft of the fibrous inner layer. A material of this nature is found to have use in the graphic arts and lithography as it can be employed as a non-abrasive, drapeable, absorbent wiper. Excessive linting from the wipe would be detrimental to the application, so increasing the level of entanglement of the surface fibers should act to decrease linting from the highly entangled surface layer, which should act as a barrier to loss of fibers or particulates form the lightly entangled core. The level of entanglement energy can be continuously varied to modify the physical properties of the wipe material to meet the required performance. It is within the scope of the present invention to control the level of entanglement in the resulting fabric to obtain materials with varying degrees of loft, absorbency, strength, and linting performance.

Nonwoven fabrics are frequently produced using staple length fibers, the fabric typically has a degree of exposed surface fibers that will lint if not sufficiently retained into the structure of the fabric. The present invention provides a finished fabric that can be cut, processed or treated, and packaged for retail sale. The cost associated with forming and finishing steps can be desirably reduced.

With reference to FIGURE 2, therein is illustrated an apparatus for practicing the present method for forming a nonwoven fabric. The fabric is formed from a fibrous batt that typically comprises natural fibers, but may comprise a synthetic staple fibers and natural/synthetic fiber blends. The fibrous batt is preferably carded and cross-lapped to form a fibrous batt, designated P. In a current embodiment, the fibrous batt comprises 100% cross-lap fibers, that is, all of the fibers of the web have been formed by cross-lapping a carded web so that the fibers are orientated at an angle relative to the machine direction of the resultant web. In this current embodiment, the fibrous batt has a draft ratio of approximately 2.8 to 1. US Patent No. 5,475,903, illustrates a web drafting apparatus.

FIGURE 2 illustrates a hydroentangling apparatus for forming nonwoven fabrics in accordance with the present invention. The apparatus includes a foraminous forming surface in the form of belt 02 upon which the fibrous batt P is positioned for pre-entangling by entangling manifold 0.1 into a wetted, lightly entangled fibrous web P'. Pre-entangling of the fibrous web is subsequently effected by movement of the web P' sequentially over a drum 10 having a foraminous forming surface, with entangling manifold 12 effecting entanglement of the web. Further entanglement of the web may be effected on the foraminous forming surface of a drum 20 by entanglement manifold 22, with the web subsequently passed over successive foraminous drums 30, 40 and 50, for successive entangling treatment by entangling manifolds 32, 42, and 51. The total optimal energy input to the fibrous batt to give the desired level of surface entanglement is in the range of about 233.4 to 350.1 J/g (0.040 to 0.060 hp-hr/lb), subject to the proviso that the hydraulic energy applied is more than 268.4 J/g (0.046 hp-hr/lb.)

The entangling apparatus of FIGURE 2 may further include an imaging and patterning drum 18 comprising a three-dimensional image transfer device for effecting imaging and patterning of the now-entangled precursor web. The image transfer device includes a moveable imaging surface which moves relative to a plurality of entangling manifolds 61, 62, 63 and 64, which act in cooperation with three-dimensional elements defined by the imaging surface of the image transfer device to effect imaging and patterning of the fabric being formed. The total energy applied to the fibrous batt of the imaging manifolds is adjusted to maintain the energy input in the range of about 233.4 to 350.1 J/g (0.040 to 0.060 hp-hr/lb), subject to the proviso that the hydraulic energy applied is more than 268.4 J/g (0.046 hp.hr/lb).

The present invention contemplates that the fibrous web P' be advanced onto the moveable imaging surface of the image transfer device at a rate which is substantially equal to the rate of movement of the imaging surface. A J-box or scray can be employed for supporting the precursor web P' as it is advanced onto the image transfer device to thereby minimize tension within the fibrous web. By controlling the rate of advancement of the fibrous batt P and the web P' through the process so as to minimize, or substantially eliminate, tension within the web, differential hydroentanglement of the fibrous web is desirably effected.

Manufacture of a durable nonwoven fabric embodying the principles of the present invention is initiated by providing the precursor nonwoven web preferably in the form of a natural and/or synthetic fibers, most preferably a cotton or cotton blend, which desirably provides good tactile and ductile softness and absorbency. During development, it was ascertained that fabric weights on the order of about 33.97 to 271.76 g/m² (1 to 8 ounces per square yard), with the range of 67.94 to 169.85 g/m² (2 to 5 ounces per square yard) being most preferred, provided the best combination of loft, softness, drapeability, absorbency, and durability.

### Examples

### Example 1

Using a forming apparatus as illustrated in FIGURE 1, a nonwoven fabric was made in accordance with the present invention by providing a fibrous batt comprising 100 weight percent cotton fiber. The fibrous batt had a basis weight of 115.49 g/m² (3.4 ounces per square yard) (plus or minus 7%). The fibrous web was 100% carded and cross-lapped, with a draft ratio of 2.8 to 1.

The fabric comprised 100 weight percent cotton as available from Barnhardt Manufacturing Company under code number RMC#2811. The fibrous batt was entangled by a series of entangling manifold stations such as diagrammatically illustrated in FIGURE 1 and in greater detail in FIGURE 2. FIGURE 2 illustrates disposition of fibrous batt P on a foraminous forming surface in the form of belt 02, with the batt acted upon by a pre-entangling manifold 01 operating at 55 bar to form a wetted and lightly entangled fibrous web. The web then passes through a series of entangling stations comprising drums having foraminous forming surfaces, for entangling by entangling manifolds, with the web thereafter directed about the foraminous forming surface of a drum 10 for entangling by entanglement manifold 12 operating at 40 bar. The web is thereafter passed over successive foraminous drums 20, 30, 40 and 50, with successive entangling treatment by entangling manifolds 22, 32, 42 and 51. In the present examples, each of the entangling manifolds included 120 micron orifices spaced at 16.65 per cm (42.3 per inch), with manifolds 22, 32, 42 and 51 successively operated at 55, 40, 55 and 0 bar, with a line of speed of 45 meters per minute. The total energy input into the fibrous batt is calculated to be 303.5 J/g (0.052 hp-hr/lb) A web having a trimmed width of 322.58 cm (127 inches) was employed.

### Comparative Example

The comparative example is selected from a commercially available product in the form of Webril 100% Cotton Handi-Pad as available from the Kendall Company. This product is formed by compression forming cotton fiber during a mercerisation process.

The accompanying Table 1 sets forth comparative test data for a fabric made by the present invention compared against a commercially available mercerised cotton fabric. Testing was done in according with the following test methods.

| **TEST** | **METHOD** |
|---|---|
| Basis weight g/m² (ounces/yd²) | ASTM D3776 |
| Bulk cm (inches) | ASTM D5729 |
| Tensiles MD and CD Grabs Kg/cm (lb/in) | ASTM D5034 |
| Elongation MD and CD Grabs (%) | ASTM D5034 |

The physical test data for Example 1 and the Comparative Example are given in , Table 1. The data in Table 1 show that the two material have similar basis weights, but the nonwoven fabric manufactured by the present invention has much greater tensile strength in both the machine and cross direction, 20 and 40 times greater, respectively, than that of the Comparative material. In addition, the tensile properties of Example 1 are more uniform when comparing the machine direction to the cross direction tensile and elongation properties.

## Claims

1. A nonwoven wipe, comprising a single fibrous batt whereupon the single fibrous batt is formed from fibers selected from 100% cotton fibers and a blend of cotton and synthetic staple length fibers, and is entangled by the application of hydraulic energy in the range of about 233.4 to 350.1 J/g (0.040 to 0.060 hp.hr/lb.) to form a differentially entangled nonwoven wipe, said nonwoven wipe having a highly entangled outer surface region and a lightly entangled inner core region, wherein said highly entangled region and said lightly entangled region are each formed from the one of said selected fibers subject to the proviso that the hydraulic energy applied is more than 268.4 J/g (0.046 hp.hr/lb.).

2. A nonwoven wipe as in claim 1, wherein the synthetic staple fibers are selected from viscose cellulose, polyacrylates, polyolefins, polyamides, polyesters and combinations thereof.

3. A nonwoven wipe as in claim 1 or 2 wherein the fabric is imaged by the application of hydraulic energy upon a three-dimensional image transfer device having a movable imaging surface.

4. A nonwoven wipe as in claim 1, 2 or 3 wherein the fabric further comprises an antimicrobial agent.

5. A nonwoven wipe as claimed in any one of claims 1 to 4, wherein the fabric further comprises an antistatic agent.

## Patentansprüche

1. Wischtuch aus Vliesstoff, das einen einzelnen Faserflor aufweist, worauf der einzelne Faserflor aus Fasern gebildet wird, die aus 100% Baumwollfasern und einer Mischung von Baumwoll- und synthetischen Stapelfasern ausgewählt werden, und durch die Anwendung von Hydraulikenergie im Bereich von etwa 233,4 bis 350,1 J/g (0,040 bis 0,060 hp.br/lb.) verwirbelt wird, um ein differentiell verwirbeltes Wischtuch aus Vliesstoff zu bilden, wobei das Wischtuch aus Vliesstoff einen stark verwirbelten Außenflächenbereich und einen schwach verwirbelten inneren Kernbereich aufweist, wobei der stark verwirbelte Bereich und der schwach verwirbelte Bereich jeweils aus der einen der ausgewählten Fasern gebildet werden, unter der Einschränkung, dass die angewandte Hydraulikenergie mehr als 268,4 J/g (0,046 hp.hr/lb.) beträgt.

2. Wischtuch aus Vliesstoff nach Anspruch 1, bei dem die synthetischen Stapelfasern unter Viskosecellulose, Polyacrylaten, Polyolefinen, Polyamiden, Polyestern und deren Kombinationen ausgewählt werden.

3. Wischtuch aus Vliesstoff nach Anspruch 1 oder 2, bei dem der Stoff durch die Anwendung von Hydraulikenergie auf einer dreidimensionalen Bildübertragungsvorrichtung mit einer beweglichen Abbildungsfläche bebildert wird.

4. Wischtuch aus Vliesstoff nach Anspruch 1, 2 oder 3, bei dem der Stoff außerdem ein antimikrobielles Mittel aufweist.

5. Wischtuch aus Vliesstoff nach einem der Ansprüche 1 bis 4, bei dem der Stoff außerdem ein Antistatilanittel aufweist.

## Revendications

1. Lingette non tissée, comprenant un unique matelas fibreux, dans laquelle l'unique matelas fibreux est formé à partir de fibres sélectionnées à partir de fibres 100% coton et d'un mélange de fibres discontinues de coton et synthétiques, et est enchevêtré par application d'énergie hydraulique dans la plage d'environ 233,4 à 350,1 J/g (de 0,040 à 0,060 hp.hr/lb.) pour former une lingette non tissée à enchevêtrements différentiels, ladite lingette non tissée ayant une région de surface extérieure très enchevêtrée et une région centrale intérieure faiblement enchevêtrée, dans laquelle ladite région très enchevêtrée et ladite région faiblement enchevêtrée sont formées chacune à partir d'une desdites fibres sélectionnées à condition que l'énergie hydraulique appliquée soit supérieure à 268,4 J/g (0,046 hp.br/lb.).

2. Lingette non tissée selon la revendication 1, dans laquelle les fibres discontinues synthétiques sont sélectionnées à partir de viscocellulose, polyacrylates, polyoléfines, polyamides, polyesters et leurs combinaisons.

3. Lingette non tissée selon la revendication 1 ou 2, dans laquelle le tissu est doté d'une image par application d'énergie hydraulique sur un dispositif de transfert d'image tridimensionnel présentant une surface mobile de formation d'image.

4. Lingette non tissée selon la revendication 1, 2 ou 3, dans laquelle le tissu comprend en outre un agent antimicrobien.

5. Lingette non tissée selon l'une quelconque des revendications 1 à 4, dans laquelle le tissu comprend en outre un agent antistatique.
